

## UNITED STATES PATENT OFFICE

2,273,731

## STAINLESS STEEL CONTAINING BISMUTH

Robert S. Peoples and Henry A. Holden Pray,  
Columbus, Ohio, assignors to Alloy Casting  
Institute, of New York, an unincorporated  
association of New York

No Drawing. Application January 17, 1940,  
Serial No. 314,244

6 Claims. (Cl. 75—126)

This invention relates to stainless irons and steels containing bismuth and more particularly to austenitic stainless steels containing a small but effective quantity of bismuth for the purpose of improving the machinability of the stainless steels and their resistance to corrosion.

We have found that the machinability of stainless steels can be materially increased by the incorporation in the stainless steels of a relatively small percentage of bismuth. As little as from 0.02 to 1% of bismuth when added to stainless steels greatly improves their machinability. We have further found that the resistance of stainless steels to the corroding action of various acids and to pitting attack in general can be materially increased by additions of bismuth.

It is therefore an important object of this invention to provide a stainless steel of improved machinability by the incorporation therein of a relatively small but effective proportion of bismuth.

It is a further important object of this invention to provide a stainless steel of improved resistance to corrosion.

Other important objects of this invention will become apparent from the following description and appended claims.

Our invention is applicable generally to any of the so-called "stainless steels," either the straight chromium or the chromium-nickel steels. We prefer, however, to employ the austenitic stainless steels, containing both chromium and nickel. Chromium may be as high as 30% and is usually present in amounts of 12% or more. The stainless steels may be either in the cast or wrought condition.

The amount of bismuth that may be added to a stainless steel to improve its machinability lies,

in general, between the limits of 0.02 and 1.0%, preferably within the narrower limits of from 0.1 to 0.6%. The bismuth can be added in any suitable manner, but most advantageously may be incorporated into the stainless steel just prior to pouring, or while in the ladle, since bismuth has a lower boiling point than the melting point of stainless steels and therefore tends to volatilize out of the molten metal, probably in the form of bismuth trioxide.

In order to incorporate as much as 0.6% of bismuth in the stainless steel, it may be necessary to add a much larger proportionate amount of bismuth in the first instance, owing to loss by volatilization. The percentages of bismuth in the stainless steel, as given herein, are those that may be found by analysis of the stainless steel. Also, while it is believed that bismuth is retained in the stainless steel largely in its elemental form, the term "bismuth" refers to the element itself, regardless of the form in which it may be present in the stainless steel.

Heats of stainless steels with and without bismuth additions have been melted and subjected to machinability tests. The tests were made by sawing and drilling the steels under rigorously controlled conditions in automatic machines. The results are expressed as a "saw index" and a "drill index." An index of 200, for example, indicates that the material machines twice as easily in that particular type of machining operation, as one whose index is 100. The remarkable and heretofore unrecognized effect of small amounts of bismuth can be seen in the data for six series of stainless and manganese steels of different types shown in Table I. The effect has further been substantiated by machine shop lathe observations.

TABLE I

## Composition

| C          | Mn        | Si        | S    | P    | Cr    | Ni   | Bi   | Saw index | Drill index |
|------------|-----------|-----------|------|------|-------|------|------|-----------|-------------|
| SERIES I   |           |           |      |      |       |      |      |           |             |
| 0.12       | 0.83      | 0.94      | 0.02 | 0.01 | 18.05 | 8.0  | 0.00 | 100       | 100         |
| SERIES II  |           |           |      |      |       |      |      |           |             |
| 0.11       | 0.82      | 0.95      | 0.02 | 0.01 | 25.0  | 12.0 | 0.00 | 100       | 100         |
| 0.11       | 0.82      | 0.95      | 0.02 | 0.01 | 25.0  | 12.0 | 0.11 | 112       | 132         |
| 0.11       | 0.82      | 0.95      | 0.02 | 0.01 | 25.0  | 12.0 | 0.13 | 133       | 147         |
| 0.13       | 0.82      | 1.15      | 0.02 | 0.01 | 25.8  | 12.2 | 0.25 | 130       | 142         |
| 0.12       | 0.83      | 1.16      | 0.02 | 0.01 | 26.6  | 12.6 | 0.37 | 140       | 265         |
| SERIES III |           |           |      |      |       |      |      |           |             |
| 0.08-0.10  | 0.75-0.85 | 0.95-1.05 | 0.03 | 0.04 | 19    | 9    | 0.00 | 100       | 100         |
| 0.08-0.10  | 0.75-0.85 | 0.95-1.05 | 0.03 | 0.04 | 19    | 9    | 0.04 | 110       | ---         |
| 0.08-0.10  | 0.75-0.85 | 0.95-1.05 | 0.03 | 0.04 | 19    | 9    | 0.08 | 108       | 183         |
| 0.08-0.10  | 0.75-0.85 | 0.95-1.05 | 0.03 | 0.04 | 19    | 9    | 0.14 | 127       | 212         |
| 0.08-0.10  | 0.75-0.85 | 0.95-1.05 | 0.03 | 0.04 | 19    | 9    | 0.19 | 134       | 313         |
| 0.08-0.10  | 0.75-0.85 | 0.95-1.05 | 0.03 | 0.04 | 19    | 9    | 0.27 | 159       | 443         |
| 0.08-0.10  | 0.75-0.85 | 0.95-1.05 | 0.03 | 0.04 | 19    | 9    | 0.32 | 161       | 411         |
| SERIES IV  |           |           |      |      |       |      |      |           |             |
| 0.095      | 0.86      | 1.03      | 0.02 | 0.01 | 19.09 | 9.01 | 0.0  | ---       | 100         |
| 0.095      | 0.86      | 1.03      | 0.02 | 0.01 | 19.09 | 9.01 | 0.59 | ---       | 193         |
| SERIES V   |           |           |      |      |       |      |      |           |             |
| 0.06       | 0.50      | 0.30      | ---- | ---- | 12.0  | 0.0  | 0.00 | 100       | ----        |
| 0.06       | 0.50      | 0.30      | ---- | ---- | 12.0  | 0.0  | 0.10 | 186       | ----        |
| SERIES VI  |           |           |      |      |       |      |      |           |             |
| 1.10       | 14.0      | 0.40      | 0.02 | 0.02 | ----  | ---- | 0.0  | 100       | ----        |
| 1.10       | 14.0      | 0.40      | 0.02 | 0.02 | ----  | ---- | 0.20 | 1,100     | ----        |

<sup>1</sup> Maximum.

It will be noted that the tests of Series VI relate to a manganese steel. Any manganese steel, that is, a steel containing between about 11 and 15% of manganese, exhibits a markedly improved machinability upon the addition thereto of a small percentage of bismuth.

Tests of samples of similar steels with and without bismuth additions indicate increased corrosion resistance when small amounts of bismuth are present. The improvement is particularly noticeable under corrosive conditions that gives rise to a "pitting" type of attack. This has been demonstrated by qualitative tests of a large number of these steels in an aqueous solution containing 5% ferric chloride and 10% sodium chloride. A 19% chromium, 9% nickel alloy is severely pitted in this solution in 2 hours. An alloy of the same composition but containing 0.30% bismuth is unattacked under the same conditions in 48 hours and one containing 0.60% bismuth is entirely immune to attack for periods in excess of a week.

The improved resistance to acid attack resulting from the addition of small amounts of bismuth to stainless steel is shown by the example of Table II.

50

TABLE II

| 55   | Composition |      |      |      |      |      |      |       | Weight loss in Mg/sq. in./day in 10% H <sub>2</sub> SO <sub>4</sub> solution, aerated and agitated, 72 hour test at 35° C. |
|------|-------------|------|------|------|------|------|------|-------|----------------------------------------------------------------------------------------------------------------------------|
|      | C           | Mn   | Si   | S    | P    | Cr   | Ni   | Bi    |                                                                                                                            |
| 0.11 | 0.82        | 0.95 | 0.02 | 0.01 | 25.0 | 12.0 | 0.00 | ----- | 372.0                                                                                                                      |
| 0.13 | 0.82        | 1.15 | 0.02 | 0.01 | 25.8 | 12.2 | 0.25 | ----- | 1.26                                                                                                                       |

60

The benefits resulting from the addition of bismuth to stainless steels are accompanied by a negligible change in the tensile properties of the steel. This is exemplified in the tensile data of Table III.

65

TABLE III

| 70     | Alloy No. | Composition |      |      |      |      |      |     |      |
|--------|-----------|-------------|------|------|------|------|------|-----|------|
|        |           | C           | Mn   | Si   | S    | P    | Cr   | Ni  | Bi   |
| 1----- | -----     | 0.08        | 0.86 | 0.85 | 0.03 | 0.04 | 19.6 | 8.9 | 0.00 |
| 2----- | -----     | 0.08        | 0.86 | 0.80 | 0.03 | 0.04 | 19.5 | 9.2 | 0.20 |
| 3----- | -----     | 0.08        | 0.86 | 0.79 | 0.03 | 0.04 | 19.3 | 9.6 | 0.20 |

75

<sup>1</sup> Maximum.

## Tensile properties (average)

| Alloy No. | Proportional limit | Yield (0.2% deforma.) | Tensile            | Elongation in 2 in. | Reduction in area |
|-----------|--------------------|-----------------------|--------------------|---------------------|-------------------|
| 1.        | P. s. i.<br>22,000 | P. s. i.<br>33,200    | P. s. i.<br>75,200 | Per cent<br>62.2    | Per cent<br>69.6  |
| 2.        | 22,000             | 33,200                | 73,500             | 59.0                | 72.3              |
| 3.        | 19,500             | 30,400                | 69,300             | 57.5                | 74.0              |

It will, of course, be understood that various details of composition may be varied through a wide range without departing from the principles of this invention and it is, therefore, not the purpose to limit the patent granted hereon otherwise than necessitated by the scope of the appended claims.

We claim as our invention:

1. A ferrous alloy containing from 0.02 to 1.0 per cent bismuth, an amount of alloying material sufficient to render the structure of the alloy austenitic and selected from the group consisting of nickel, nickel and chromium, and manganese, and the remainder substantially all iron, said bismuth content effectively improving machinability of the alloy.

2. An alloy having improved machinability con-

taining 12 to 30 per cent chromium, 0.02 to 1.0 per cent bismuth, and the remainder substantially all iron.

3. An alloy having improved machinability containing 12 to 30 per cent chromium, 8 to 12.6 per cent nickel, 0.02 to 1.0 per cent bismuth, and the remainder substantially all iron.

4. An austenitic steel alloy having improved machinability containing 11 to 15 per cent manganese, 0.02 to 1.0 per cent bismuth, and the remainder substantially all iron.

5. A ferrous alloy of the stainless steel type containing between 12 and 30 per cent chromium, and having improved machinability due to the presence of bismuth therein, said alloy containing from .02 to 1.0 per cent bismuth.

6. A ferrous alloy containing an amount of alloying material sufficient to render the structure of said alloy austenitic and selected from the group consisting of nickel, nickel and chromium, and manganese, and containing from 0.02 to 1.0 per cent bismuth, said alloy having improved machinability due to the said presence of bismuth therein.

ROBERT S. PEOPLES.  
HENRY A. HOLDEN PRAY.